

May 23, 1961

D. H. WILLSON ET AL

2,985,586

HYDROFINING OF LUBRICATING OIL FRACTIONS

Filed Nov. 26, 1958



FIG. 1.

EFFECT OF WEIGHT PER CENT SULFUR AND HYDROFINING TEMPERATURE ON AVERAGE BEARING WEIGHT LOSS AND PISTON SKIRT VARNISH FOR PANHANDLE 150 - NEUTRAL OIL

FIG. 2.



INVENTORS.

DAN H. WILLSON,  
GEORGE R. L. SHEPHERD,

BY

*James B. McDaniel*  
ATTORNEY.

1

2,985,586

## HYDROFINING OF LUBRICATING OIL FRACTIONS

Dan H. Willson, Houston, and George R. L. Shepherd, Baytown, Tex., assignors, by mesne assignments, to Esso Research and Engineering Company, Elizabeth, N.J., a corporation of Delaware

Filed Nov. 26, 1958, Ser. No. 781,419

7 Claims. (Cl. 208—264)

The present invention is directed to hydrofining of lubricating oil fractions. More particularly, the invention is concerned with treating a lubricating oil fraction in the presence of hydrogen to form an improved lubricant. In its more specific aspects, the invention is concerned with the formation of a lubricating oil which contains sulfur.

The present invention is directed to the production of improved lubricating oil in which a lubricating oil fraction is hydrofined in the presence of a sulfur-resistant catalyst at a temperature within the range from about 400° to about 650° F. under a pressure within the range from about 200 to about 1,000 pounds per square inch and at a space velocity within the range from about 1 to about 10 v./v./hr. in the presence of sufficient free hydrogen-containing gas to provide from about 50 to about 5,000 standard cubic feet of hydrogen per barrel of the lubricating oil fraction, the hydrogen-containing gas also containing from about 5% to about 95% by volume of hydrogen sulfide to form a product containing sulfur and of improved lubricating quality.

The feed stock employed in the present invention is a lubricating oil fraction which may boil in the range from about 800° to about 1,200° F. and ordinarily will comprise a fraction of crude petroleum. Higher boiling fractions may also be used. Such lubricating oil fractions are known as neutral oils, light motor oils, medium motor oils, and bright stocks. It is contemplated that the lubricating oil fraction employed in the present invention may suitably be a solvent raffinate of a lubricating oil fraction obtained from crude petroleum. Examples of the crude petroleum from which the lubricating oil fraction may be obtained are the Gulf Coastal crudes, Panhandle crudes, Pennsylvania type crude oils, and California crude oils and the like.

The invention is suitably practiced with a suitable sulfur-resistant catalyst, of which many are known to the art. As examples of suitable catalysts are the oxides and sulfides of metals such as vanadium, chromium, manganese, iron, cobalt, nickel, molybdenum, tungsten, and the like. Specific examples of such catalysts are cobalt molybdate, nickel-tungsten sulfide, cobalt sulfide, molybdenum sulfide, molybdenum oxide, nickel sulfide, tin sulfide, and the like. The catalysts are preferably employed on a support or a suitable carrier such as alumina, magnesia, silica, zirconia, spinels, and the like. The catalyst may be employed as a fixed bed catalyst, in the form of a fluidized bed, or as a slurry in the lubricating oil, or in any other suitable manner.

The present invention is suitably conducted in the presence of hydrogen, and an amount of hydrogen within the range from about 50 to about 5,000 standard cubic feet per barrel is employed. A preferred amount of hydrogen is from about 65 to about 500 standard cubic feet per barrel. The hydrogen for the operation is provided by charging a hydrogen-containing gas to the catalyst along with the feed stock. The hydrogen-containing gas may be added from an extraneous source and may be pure hydrogen or may comprise a mixture of hydro-

2

gen and gaseous material such as light hydrocarbons. For example, gaseous material from the operation may provide at least a part of the hydrogen-containing gas as a source of the hydrogen for the reaction.

- 5 The amount of hydrogen sulfide which is added with the hydrogen is within the range from about 5% to about 95% by volume of the total gas with a preferred range from about 20% to about 70% by volume based on the total gas. In the present invention the hydrogen sulfide 10 may largely be provided from an extraneous source since ordinarily the amount of hydrogen sulfide provided in a hydrofining operation is not sufficient for best results. However, recycle of tail gas may provide sufficient hydrogen sulfide build up.
- 15 The temperatures employed in the practice of the present invention may suitably range from about 400° to about 650° F. with desirable results being obtained at about 500° F. A preferred temperature range is from about 475° to about 575° F.
- 20 Pressures may suitably range from about 200 to about 1,000 pounds per square inch with good results being obtained at about 750 pounds per square inch. A preferred range is from about 400 to about 800 pounds per square inch.
- 25 The space velocity may range from about 1 to about 10 volumes of feed per volume of catalyst per hour with a preferred space velocity from about 3 to about 5 v./v./hr.
- 30 In accordance with the present invention, improved results are obtained in that the present invention provides a lubricating oil product which contains sulfur in an amount greater than that usually present in a hydrofined lubricating oil product. The presence of sulfur confers unusual properties on the lubricating oil in that in the 35 present invention the response of the product to lubricating oil additives and inhibitors is enhanced. In other words, for a given amount of a lubricating oil additive or inhibitor, a greater response is had with the product of the present invention than with a conventionally hydrofined product. Furthermore, the product hydrofined according to this invention performs more satisfactorily than conventionally hydrofined products without inhibitors. This means that with the present invention, amounts of additives can be reduced and yet obtain beneficial results.
- 40 The present invention will be further illustrated by reference to the drawing in which:
- 45 Fig. 1 is a flow diagram of a preferred mode of practicing the invention, and
- 50 Fig. 2 is a graphical presentation of data showing the effect of sulfur and hydrofining temperature on bearing weight loss and piston skirt varnish for a Panhandle 150 neutral oil.
- 55 Referring now to the drawing and particularly to Fig. 1, numeral 11 designates a charge line by way of which a lubricating oil fraction is introduced into the system from a source not shown. This lubricating oil fraction may suitably be a phenol raffinate of a petroleum lubricating oil fraction. The fraction charged by line 11 may 60 suitably be and preferably is either a neutral oil, light motor oil, medium oil, or a bright stock, or the total fraction may be charged. For purposes of this description only, a neutral or light motor oil is charged. Introduced into line 11 by line 12 is a hydrogen-containing gas in which hydrogen sulfide is suitably added by way 65 of line 13 controlled by valve 14. The mixture of hydrogen, hydrogen sulfide, and lubricating oil is suitably introduced into a heater 15 provided with a heating coil 16 and with burners such as gas burners 17, by way of which the temperature of the mixture is raised to a temperature within the range given before. The heated mixture, under the conditions set out herein, is discharged from heater 15 by line 18 and introduced thereby into a reaction zone 70

19 containing a bed of catalyst 20 such as cobalt molybdate. Under the conditions for the practice of this invention, the lubricating oil fraction is suitably hydrofined and a product is formed which is withdrawn by line 21 and discharged thereby into a separation zone 22, which is of suitable capacity to provide a residence time for separation of normally gaseous products from the liquid products, the gaseous products being withdrawn from separation zone 22 by line 23 for recycling to line 12 by branch line 24 controlled by valve 25. This recycled gas provides at least a portion of the hydrogen and may provide a portion of the hydrogen sulfide for the process. A portion of the gas may suitably be discharged from line 23 by manipulation of valve 26.

When the total lubricating oil fraction is charged, the liquid products from zone 22 are withdrawn therefrom by line 27 and introduced into a fractional distillation zone 28, which is shown as a single fractional distillation tower but which may be a plurality of fractional distillation towers, each equipped with all auxiliary apparatus usually incident to a modern fractional distillation tower. Thus, zone 28 is provided with suitable internal, vapor-liquid contacting means, cooling and condensing means, means for inducing reflux and the like, not shown. Zone 28 is equipped with a heating means 29, illustrated by a steam coil, for adjusting temperature and pressure for distillation of the liquid product. Line 30 is provided for removal of light fractions boiling above lubricating oil and lines 31, 32, and 33 controlled, respectively, by valves

34, 35, and 36 for withdrawal and recovery of the lubricating oil fractions. Line 37 is provided for discharge of heavier fractions which may be of bright stock quality. It will be understood, however, that when one of the 5 components of the total lubricating oil fraction is charged, zone 28 may be used only to remove light ends and to recover the desired product through line 37 with lines 31, 32, and 33 being closed. While the inhibitor may be added directly to the distilled product, the inhibitor 10 is preferably added to the final blended motor oil.

Since the product of this operation has enhanced response to lubricating oil additives or inhibitors, provision is made for adding a lubricating oil additive by way of manifold 38 which connects into lines 31, 32, and 33 and 15 into which flow is controlled by way of valves 39, 40, and 41 as may be desired. Where a selected oil such as neutral oil is hydrofined and withdrawn by line 37, inhibitor may be added thereto as desired.

If the recycled gas does not provide sufficient hydrogen, this may be provided from an extraneous source by opening valve 42 in line 12.

In order to illustrate the present invention further, a number of hydrofining runs were made employing Panhandle 150-neutral raffinate, Panhandle light motor oil 25 raffinate, and Panhandle 150-X bright stock raffinate using 10 to 20 mesh cobalt molybdate as a catalyst.

The following table I sets out the several conditions and the product inspections resulting from the hydrofining operations.

TABLE I  
Hydrofining conditions and product inspections

| Type of Catalyst                                       | Cobalt Molybdate, 10-20 Mesh |                              |        |        |        |        |        |        |        |        |        |        |        |        |
|--------------------------------------------------------|------------------------------|------------------------------|--------|--------|--------|--------|--------|--------|--------|--------|--------|--------|--------|--------|
|                                                        | Feed                         | 465                          | Feed   | 474    | 475    | 476    | 477    | 478    | 498    | 499    | Feed   | 527    | 528    | 529    |
| Feed Stocks                                            |                              |                              |        |        |        |        |        |        |        |        |        |        |        |        |
| Reactor Temperature, ° F                               |                              | 475                          | -----  | 500    | 500    | 475    | 475    | 550    | 575    | 550    | -----  | 475    | 500    | 550    |
| Reactor Pressure, P.s.i.g.                             |                              | 300                          | -----  | 750    | 750    | 700    | 700    | 750    | 750    | 750    | -----  | 750    | 750    | 750    |
| Feed Rate, v.v./Hr.                                    | 3.1                          | -----                        | 3.2    | 3.1    | 3.2    | 3.2    | 3.2    | 4.8    | 5.0    | 5.0    | -----  | 3.3    | 3.3    | 3.2    |
| Total Gas Rate, s.c.f./Hr.                             | 27                           | -----                        | 24     | 26     | 26     | 24     | 30     | 23     | 23     | 23     | -----  | 22     | 26     | 23     |
| Hydrogen Sulfide Injected, Volume Percent of Total Gas |                              | 11                           | -----  | 5      | 11     | 10     | 5      | 22     | 68     | 68     | -----  | 60     | 66     | 79     |
| Hydrogen Gas:                                          |                              |                              |        |        |        |        |        |        |        |        |        |        |        |        |
| Volume Percent of Total Gas                            |                              | 89                           | -----  | 95     | 89     | 90     | 95     | 78     | 32     | 32     | -----  | 40     | 34     | 21     |
| S.c.f./Bbl. Feed                                       |                              | 342                          | -----  | 337    | 345    | 340    | 339    | 339    | 71     | 69     | -----  | 126    | 126    | 72     |
| Product Inspections:                                   |                              |                              |        |        |        |        |        |        |        |        |        |        |        |        |
| Gravity, ° API                                         | 33.2                         | 33.3                         | 32.4   | 32.6   | 32.6   | 32.6   | 32.6   | 32.7   | 32.7   | 32.7   | 33.1   | 33.0   | 33.0   | 33.1   |
| Flash, O.C. ° F                                        | 400                          | 415                          | 430    | 425    | 425    | 425    | 425    | 410    | 420    | 420    | 415    | 405    | 410    | 410    |
| Viscosity, SSU/100° F                                  | 139.6                        | 137.7                        | 148.0  | 146.3  | 146.1  | 146.5  | 146.4  | 146.2  | 146.4  | 146.0  | 141.7  | 142.0  | 141.7  | 139.7  |
| Viscosity, SSU/210° F                                  | 42.9                         | 42.8                         | 43.4   | 43.2   | 43.3   | 43.3   | 43.2   | 43.3   | 43.3   | 43.3   | 43.3   | 42.9   | 43.0   | 42.8   |
| Color, Tag Robinson                                    | 9/4                          | 19 1/4                       | 9 1/2  | 19 3/4 | 18 1/2 | 19     | 18 1/2 | 19 1/2 | 19 1/2 | 19     | 21     | 10 1/4 | 19     | 21 1/4 |
| Color Hold Tag Robinson                                |                              | 17 1/2                       | 9 1/2  | 19     | 18     | 18 1/2 | 18     | 19 1/2 | 19     | 20 1/2 | -----  | 18 1/2 | 19 1/2 | 21     |
| Pour, ° F                                              | 15                           | 15                           | 15     | 25     | 20     | 20     | 25     | 30     | 30     | 30     | 10     | 10     | 15     | 25     |
| Cloud, ° F                                             | 16                           | 24                           | 24     | 30     | 26     | 28     | 28     | 42     | 44     | 45     | 20     | 16     | 25     | 28     |
| Sulfur, Wt. percent                                    | 0.21                         | 0.20                         | 0.27   | 0.14   | 0.16   | 0.20   | 0.19   | 0.10   | 0.14   | 0.18   | 0.24   | 0.28   | 0.27   | 0.16   |
| Con. Carbon, Wt. percent                               | 0.01                         | 0.05                         | 0.01   | 0.01   | 0.01   | 0.01   | 0.01   | 0.01   | 0.00   | 0.00   | 0.00   | 0.00   | 0.00   | 0.00   |
| Aniline Point, ° F                                     | 224                          | 222                          | 220    | 221    | 221    | 221    | 221    | 221    | 221    | 221    | 221    | 221    | 221    | 222    |
| Type of Catalyst                                       |                              |                              |        |        |        |        |        |        |        |        |        |        |        |        |
| Run Number                                             |                              | Cobalt Molybdate, 10-20 Mesh |        |        |        |        |        |        |        |        |        |        |        |        |
| Feed Stocks                                            |                              | Feed                         | 479    | 480    | 481    | 382    | 494    | 495    | 500    | 501    |        |        |        |        |
| Panhandle Light Motor Raffinate                        |                              |                              |        |        |        |        |        |        |        |        |        |        |        |        |
| Reactor Temperature, ° F                               |                              |                              | 500    | 500    | 425    | 425    | 575    | 575    | 575    | 575    | 625    |        |        |        |
| Reactor Pressure, P.s.i.g.                             |                              |                              | 700    | 700    | 700    | 700    | 750    | 750    | 750    | 750    | 750    |        |        |        |
| Feed Rate, v.v./hr.                                    | 3.1                          |                              | 3.1    | 3.1    | 3.1    | 3.1    | 3.1    | 3.1    | 3.1    | 3.1    | 4.7    |        |        |        |
| Total Gas Rate, s.c.f./hr.                             | 24                           |                              | 26     | 26     | 26     | 25     | 28     | 28     | 35     | 35     | 23     |        |        |        |
| Hydrogen Sulfide Injected, Volume Percent of Total Gas |                              |                              | 5      | 11     | 12     | 6      | 50     | 60     | 68     | 70     |        |        |        |        |
| Hydrogen Gas:                                          |                              |                              |        |        |        |        |        |        |        |        |        |        |        |        |
| Volume Percent of Total Gas                            |                              |                              | 95     | 89     | 88     | 94     | 50     | 40     | 32     | 30     | 30     |        |        |        |
| S.c.f./Bbl. Feed                                       |                              |                              | 347    | 349    | 346    | 349    | 212    | 212    | 72     | 72     | 72     |        |        |        |
| Product Inspections:                                   |                              |                              |        |        |        |        |        |        |        |        |        |        |        |        |
| Gravity, ° API                                         | 30.7                         | 30.9                         | 30.9   | 30.7   | 30.8   | 31.0   | 31.0   | 31.0   | 31.0   | 31.0   | 31.0   |        |        |        |
| Flash, O.C. ° F                                        | 465                          | 460                          | 470    | 470    | 465    | 455    | 450    | 455    | 455    | 455    | 455    |        |        |        |
| Viscosity, SSU/100° F                                  | 324                          | 316                          | 318    | 323    | 322    | 311    | 311    | 311    | 312    | 312    | 306    |        |        |        |
| Viscosity, SSU/210° F                                  | 54.6                         | 54.2                         | 54.3   | 54.7   | 54.6   | 54.0   | 54.1   | 54.1   | 54.1   | 54.1   | 53.7   |        |        |        |
| Color, Tag Robinson                                    | 5                            | 13                           | 12     | 10     | 10     | 17 1/2 | 17 1/2 | 17 1/2 | 17 1/2 | 17 1/2 | 14 1/2 |        |        |        |
| Color Hold Tag Robinson                                |                              | 12                           | 11 1/2 | 9 1/2  | 9 1/2  | 17 1/2 | 17 1/2 | 17 1/2 | 17 1/2 | 17 1/2 | 13 1/2 |        |        |        |
| Pour, ° F                                              | 15                           | 25                           | 25     | 20     | 20     | 35     | 35     | 35     | 35     | 35     | 35     |        |        |        |
| Cloud, ° F                                             | 20                           | 26                           | 28     | 22     | 26     | 45     | 45     | 45     | 42     | 42     | 40     |        |        |        |
| Sulfur, Wt. percent                                    | 0.32                         | 0.22                         | 0.24   | 0.33   | 0.33   | 0.18   | 0.18   | 0.18   | 0.18   | 0.18   | 0.18   |        |        |        |
| Con. Carbon, Wt. Percent                               | 0.04                         | 0.04                         | 0.04   | 0.02   | 0.04   | 0.02   | 0.02   | 0.02   | 0.02   | 0.02   | 0.02   |        |        |        |
| Aniline Point, ° F                                     | 231                          | 232                          | 232    | 232    | 231    | 234    | 234    | 234    | 234    | 234    | 234    |        |        |        |

TABLE I—Continued  
*Hydrofining conditions and product inspections—Continued*

| Type of Catalyst                                       | Cobalt Molybdate, 10-20 Mesh           |       |                  |                  |                  |       |       |                  |                  |                  |                  |                  |
|--------------------------------------------------------|----------------------------------------|-------|------------------|------------------|------------------|-------|-------|------------------|------------------|------------------|------------------|------------------|
|                                                        | Feed                                   | 483   | 484              | 485              | 486              | 496   | 497   | Feed             | 521              | 522              | 525              | 526              |
| Run Number                                             | Panhandle 150-X Bright Stock Raffinate |       |                  |                  |                  |       |       |                  |                  |                  |                  |                  |
| Feed Stocks                                            |                                        |       |                  |                  |                  |       |       |                  |                  |                  |                  |                  |
| Reactor Temperature, °F                                |                                        | 500   | 500              | 550              | 600              | 575   | 575   |                  | 450              | 500              | 500              | 450              |
| Reactor Pressure, P.s.i.g.                             |                                        | 700   | 700              | 700              | 700              | 750   | 750   |                  | 750              | 750              | 750              | 750              |
| Feed Rate, v.v./hr.                                    | 3.1                                    | 3.0   | 3.0              | 3.0              | 2.9              | 4.3   |       | 3.1              | 3.2              | 3.2              | 3.2              | 3.2              |
| Total Gas Rate, S.c.f./Hr.                             | 24                                     | 26    | 29               | 29               | 36               | 30    |       | 14               | 14               | 20               | 20               | 20               |
| Hydrogen Sulfide Injected, Volume Percent of Total Gas |                                        | 5     | 11               | 22               | 22               | 61    | 76    |                  | 0                | 0                | 28               | 30               |
| Hydrogen Gas:                                          |                                        |       |                  |                  |                  |       |       |                  |                  |                  |                  |                  |
| Volume Percent of Total Gas                            | 95                                     | 89    | 78               | 78               | 39               | 24    |       | 100              | 100              | 72               | 70               | 70               |
| S.c.f./Bbl. Feed                                       | 349                                    | 353   | 362              | 356              | 224              | 80    |       | 207              | 206              | 206              | 206              | 206              |
| Product Inspections:                                   |                                        |       |                  |                  |                  |       |       |                  |                  |                  |                  |                  |
| Gravity, °API                                          | 27.4                                   | 27.3  | 27.3             | 27.5             | 27.7             | 27.4  | 27.4  | 27.5             | 27.5             | 27.5             | 27.5             | 27.5             |
| Flash, O. C. °F                                        | 595                                    | 590   | 590              | 570              | 570              | 565   | 580   | 575              | 570              | 570              | 575              | 575              |
| Viscosity, SSU/100° F                                  | 2,410                                  | 2,382 | 2,422            | 2,324            | 2,258            | 2,350 | 2,333 | 2,120            | 2,094            | 2,064            | 2,090            | 2,113            |
| Viscosity, SSU/210° F                                  | 157.2                                  | 155.7 | 155.9            | 154.4            | 151.3            | 153.7 | 154.7 | 145.0            | 143.8            | 142.2            | 143.8            | 144.7            |
| Color, Tag Robinson                                    | 2 <sup>1/2</sup>                       | 4     | 4 <sup>1/2</sup> | 4 <sup>1/2</sup> | 5 <sup>1/2</sup> | +9+   | +9+   | 2 <sup>1/2</sup> | 3                | 4 <sup>1/2</sup> | 5 <sup>1/2</sup> | 4                |
| Color Hold Tag Robinson                                | 2 <sup>1/2</sup>                       | 3     | 3 <sup>1/2</sup> | 3 <sup>1/2</sup> | 4 <sup>1/2</sup> | +9+   | +9+   | 2                | 1 <sup>1/2</sup> | 3 <sup>1/2</sup> | 4 <sup>1/2</sup> | 3 <sup>1/2</sup> |
| Pour, °F                                               | 20                                     | 20    | 20               | 25               | 30               | 30    | 25    | 15               | 15               | 15               | 10               | 15               |
| Cloud, °F                                              | 22                                     | 18    | 18               |                  |                  |       | 52    | 50               | 26               | 28               | 31               | 29               |
| Sulfur, Wt. Percent                                    | 0.47                                   | 0.45  | 0.46             | 0.42             | 0.29             | 0.42  | 0.43  | 0.48             | 0.47             | 0.36             | 0.45             | 0.47             |
| Con. Carbon, Wt. Percent                               | 0.64                                   | 0.70  | 0.72             | 0.59             | 0.56             | 0.68  | 0.74  | 0.64             | 0.70             | 0.73             | 0.63             | 0.65             |
| Aniline Point, °F                                      | 261                                    | 261   | 264              | 264              | 264              | 262   | 262   | 260              | 260              | 260              | 260              | 260              |

Selected products from the several runs illustrated in Table I were then subjected to a 36-hour L-4 Chevrolet engine test and these products were compared with similar products produced by clay contacting only and with lubricating oils hydrofined in the absence of hydrogen sulfide in the entering gas. In Table II the test results in Panhandle 150 neutral oils of Table I are presented.

that samples SX-4803 and 4804 where the present invention was also practiced had higher sulfur contents than the conventionally hydrofined oils of SX-4400. Sample SX-5479, on the other hand, had a piston skirt varnish which was substantially the same as that of the clay-contacted oil and had a lower average bearing weight loss than any of the oils and yet the sulfur content of

TABLE II  
*36-hour, L-4 Chevrolet engine test results on Panhandle 150-neutral*

| Sample Number                                   | SX-4174 | SX-4400 | SX-4401 | SX-4577 | SX-4505 | SX-4803 |
|-------------------------------------------------|---------|---------|---------|---------|---------|---------|
| Hydrofining Temp., °F                           | (2)     | 575     | 575     | 575     | 475     | 500     |
| Hydrofiner Run Number                           |         | 413     | 413     | 465     | 474     |         |
| Percent in Entering Gas                         | 0       | 0       | 0       | 11      | 5       |         |
| Wt. Percent Sulfur (Before Additive)            | 0.22    | 0.04    | 0.04    | 0.04    | 0.20    | 0.14    |
| Additive                                        | 0       | 0       | 0.5%    | 0.7%    | 0       | 0       |
| 36-Hr., L-4 Results:                            |         |         |         |         |         |         |
| Piston Skirt SRI (Southwest Research Institute) | 8.8     | 6.1     | 6.1     | 0.1     | 6.8     | 5.8     |
| Varnish, Total                                  | 46.3    | 40.1    | 40.6    | 46.6    | 43.8    | 42.3    |
| Sludge, Total                                   | 47.5    | 46.0    | 48.0    | 48.0    | 46.5    | 45.0    |
| Avg. BWL, gms                                   | 0.728   | 2.854   | 1.233   | 0.015   | 1.032   | 1.627   |
| Used Oil Data (36-Hrs.):                        |         |         |         |         |         |         |
| Percent Viscosity Increase SSU/100° F           | 23.3    | 30.9    | 3.12    |         |         | 46.1    |
| Sample Number                                   | SX-4804 | SX-5150 | SX-4962 | SX-5479 | SX-4805 | SX-4806 |
| Hydrofining Temp., °F                           | 550     | 550     | 575     | 500     | 475     | 550     |
| Hydrofiner Run Number                           | 478     | 499     | 498     | 528     | 476     | 478     |
| Percent H <sub>2</sub> S in Entering Gas        | 22      | 68      | 68      | 66      | 10      | 22      |
| Wt. Percent Sulfur (Before Additive)            | 0.10    | 0.18    | 0.14    | 0.27    | 0.20    | 0.10    |
| Additive                                        | 0       | 0       | 0       | 0       | 0.5%    | 0.5%    |
| 36-Hr., L-4 Results:                            |         |         |         |         |         |         |
| Piston Skirt SRI (Southwest Research Institute) | 5.4     | 7.7     | 8.3     | 8.5     | 8.2     | 9.5     |
| Varnish, Total                                  | 39.4    | 43.7    | 45.8    | 46.0    | 45.7    | 46.0    |
| Sludge, Total                                   | 44.0    | 45.0    | 47.5    | 47.5    | 47.5    | 48.0    |
| Avg. BWL, gms                                   | 1.997   | 0.820   | 1.632   | 0.458   | 0.092   | 0.020   |
| Used Oil Data (36-Hrs.):                        |         |         |         |         |         |         |
| Percent Viscosity Increase, SSU/100° F          | 53.7    | 38.3    | 31.2    | 18.7    | 15.7    | 15.7    |

<sup>1</sup> Zinc dialkyl dithiophosphate.

<sup>2</sup> Clay contacted.

Referring to Table II, it will be seen that sample No. SX-4962 has a piston skirt varnish of nearly equal quality to that of SX-4174, where the oil was finished by clay contacting. In this rating, the higher the value, the better the rating. Furthermore, SX-4962 is of better quality than the conventionally hydrofined oil as represented by SX-4400. It is to be noted that the sulfur content of the conventionally hydrofined oil of SX-4400. It is to be noted that the sulfur content of sample SX-4962 is greater than the sulfur content of the conventionally hydrofined oil of SX-4400. It is to be further noted

this fraction is substantially greater than any of the oils.

As stated before, hydrofining in accordance with the present invention improves the additive response of the oil when compared to conventional hydrofining. Again referring to Table II and specifically to samples SX-4401, 4577, and 4806, it will be clear that the additives response of the conventionally hydrofined oil SX-4401 was not as great as SX-4806, representing the present invention. Comparing SX-4806 with SX-4577, where a greater amount of additive was used, it will be used that a higher piston skirt varnish was obtained with the pres-

ent invention than where a greater amount of additive was used in a conventionally hydrofining product. It may be seen from the data of Table II that at the preferred hydrofining temperature, a lesser amount may be sufficient to give the same quality as was obtained with 0.5% as in SX-4806. Hence, the additive requirements might be reduced anywhere from about 50% to about 85% by the practice of the present invention.

obtained with a conventional hydrofined product. By providing hydrogen sulfide in the inlet gas, it is possible to substantially improve the quality of the lubricating oil and increase its response to additives.

The nature and objects of the present invention having been completely described and illustrated, what we wish to claim as new and useful and secure by Letters Patent is:

1. A method for producing an improved lubricating oil

TABLE III  
36 hour, L-4 Chevrolet engine test results on Panhandle  
LMO

| Sample Number                            | SX-3922                  | SX-3923 | SX-3924 | SX-4963 | SX-4019 | SX-4145 |
|------------------------------------------|--------------------------|---------|---------|---------|---------|---------|
| Hydrofining Temp., ° F.                  | 625                      | 425     | 425     | 625     | 425     | 425     |
| Hydrofiner Run Number                    | Clay<br>Contacted<br>351 | 383     | 481     | 351     | 383     |         |
| Percent H <sub>2</sub> S in Entering Gas | 0                        | 0       | 12      | 0       | 0       | 0       |
| Wt. Percent Sulfur (before additive)     | 0.29                     | 0.02    | 0.25    | 0.34    | 0.02    | 0.25    |
| Additive                                 | 0                        | 0       | 0       | 0       | +0.5%   | +0.5%   |
| 36-Hr., L-4 Results:                     |                          |         |         |         |         |         |
| Piston Skirts, SRI                       | 9.5                      | 9.3     | 9.0     | 9.2     | 9.1     | 9.5     |
| Varnish, Total                           | 47.5                     | 47.3    | 47.0    | 47.2    | 47.1    | 47.5    |
| Sludge, Total                            | 48.0                     | 48.0    | 47.5    | 48.0    | 48.0    | 48.5    |
| Avg. B.W.L. gms                          | 0.669                    | 3.163   | 0.893   | 0.698   | 0.587   | 0.054   |
| Used Oil Data (36-Hrs.):                 |                          |         |         |         |         |         |
| Percent Viscosity Increase—              |                          |         |         |         |         |         |
| SSU/100° F                               | 17.4                     | 52.6    | 22.9    | 19.8    | 27.7    | 7.2     |
| SSU/210° F                               | 6.1                      | 21.7    | 8.2     | 6.8     | 8.4     | 3.3     |

<sup>1</sup> Zinc dialkyl dithiophosphate.

In order to show the improved results further, referring to Table III, it will be seen that oils of a quality substantially identical with clay-contacted produced oils are obtained. Comparing SX-3922 with SX-4963, which represents the present invention, the product of the present invention was substantially the same as the clay-contacted oil comparing the clay-contacted oil, as represented by SX-3922, and the oil produced in accordance with this operation, SX-4963, with SX-3924, which is the conventionally produced oil, it will be seen that the practice of the present invention produces an oil which has a lower bearing weight loss and a higher sulfur content.

Referring to Fig. 2, the sulfur content of the Panhandle 150-neutral is plotted against piston skirt varnish rating and average bearing weight loss. These data show that the bearing weight loss decreases as sulfur content of the hydrofined product increases and that the piston skirt varnish rating is dependent on the sulfur content and the hydrofining temperature. By way of explanation as stated supra, a low bearing weight loss and a high piston skirt varnish rating are desirable.

From these results, it is clear that the present invention gives substantially improved results over conventional hydrofining operations where hydrogen sulfide is not employed in the hydrogen-containing gas.

The lubricating oil additives employed in the practice of the present invention may suitably include the well-known lubricating oil antioxidants and corrosion inhibitors, such as described by Kalichevsky and Kobe in their work "Petroleum Refining with Chemicals," Elsevier Publishing Co., New York, 1956, in Tables 159 and 166. Examples of such compounds are barium salt of alkyl phenol sulfide, cadmium, copper, or lead oleate or naphthenate, copper compounds, calcium salt of alkyl phenol sulfides or disulfides, metal alkyl xanthates, alkaline earth and alkaline metal salts of mahogany acids, aluminum diphenate, aluminum naphthenate, bivalent metal sulfonates, and the like. It is contemplated that these additives and those mentioned by Kalichevsky et al. supra may be employed in the practice of the present invention.

These several antioxidants and corrosion inhibitors are given by way of illustration and not by way of limitation.

In the practice of the present invention, the sulfur content of the hydrofined product is greater than that

30 which comprises hydrofining a lubricating oil fraction in the presence of a sulfur-resistant catalyst at a temperature within the range from about 400° to about 575° F. under a pressure within the range from about 200 to about 1,000 pounds per square inch and at a space velocity within the range from about 1 to about 10 v./v./hr. in 35 the presence of sufficient free hydrogen-containing gas to provide from about 50 to about 5,000 standard cubic feet of hydrogen per barrel of said lubricating oil fraction, said gas also containing from about 5% to about 95% by volume of hydrogen sulfide, to form a product containing an increased amount of sulfur and of improved lubricating quality over conventionally hydrofined oils.

2. A method in accordance with claim 1 in which the catalyst is cobalt molybdate.

3. A method in accordance with claim 1 in which an inhibitor is added to the product.

4. A method in accordance with claim 1 in which the lubricating oil fraction is obtained from Panhandle crude.

5. A method for producing an improved lubricating oil 50 which comprises hydrofining a lubricating oil fraction in the presence of cobalt molybdate at a temperature within the range from about 475° to about 575° F. under a pressure within the range from about 400 to about 800 pounds per square inch and at a space velocity within the range from about 3 to about 5 v./v./hr. in the presence of sufficient free hydrogen-containing gas to provide from about 65 to about 500 standard cubic feet of hydrogen per barrel of said lubricating oil fraction, said gas also containing from about 20 to about 95% by volume of hydrogen sulfide to form a product containing an increased amount of sulfur and of improved lubricating quality over conventionally hydrofined oils.

6. An improved lubricating oil containing sulfur formed by hydrofining a lubricating oil fraction in the presence of a sulfur resistant catalyst at a temperature within the range from about 400° to about 575° F. under a pressure within the range from about 200 to about 1,000 pounds per square inch and at a space velocity within the range from about 1 to about 10 v./v./hr. in the presence of sufficient free hydrogen-containing gas to provide from about 50 to about 500 standard cubic feet of hydrogen per barrel of said lubricating oil fraction, said gas also containing from about 5% to about 95% by volume of hydrogen sulfide.

7. An improved lubricating oil in accordance with claim

6 in which the lubricating oil fraction is derived from Panhandle crude.

References Cited in the file of this patent

UNITED STATES PATENTS

2,567,252 Strang Sept. 11, 1951  
2,638,438 Hoffmann et al. May 12, 1953

5 2,669,560  
2,706,167  
2,763,358  
2,817,653  
2,822,332  
2,865,850  
2,914,470

|                |                |
|----------------|----------------|
| Sperry         | Feb. 16, 1954  |
| Harper et al.  | Apr. 12, 1955  |
| Linn et al.    | Sept. 18, 1956 |
| Cole et al.    | Dec. 24, 1957  |
| Logan          | Feb. 4, 1958   |
| Holcomb et al. | Dec. 23, 1958  |
| Johnson et al. | Nov. 24, 1959  |